# EUROPEAN PATENT SPECIFICATION

(11) **EP 0 277 018 B1**
(45) Date of publication and mention of the grant of the patent: **01.04.1992**
(21) Application number: 88300727.0
(22) Date of filing: 28.01.1988
(51) Int. Cl.: C10L 9/10

(54) **Water absorbing polymers**
Wasseradsorbierende Polymere
Polymères adsorbant l'eau

(30) Priority: 30.01.1987 GB 8702052; 20.07.1987 GB 8717093; 13.08.1987 GB 8719215; 13.08.1987 GB 8719216
(43) Date of publication of application: 03.08.1988
(73) Proprietor: ALLIED COLLOIDS LIMITED, Bradford, West Yorkshire BD12 0JZ (GB)
(72) Inventor: Farrar, David, Bradford, West Yorkshire (GB); Flesher, Peter, Bingley, West Yorkshire (GB); Skinner, Malcolm, Bradford, West Yorkshire (GB)
(74) Representative: Lawrence, Peter Robin Broughton

(56) References cited:
- EP-A- 0 161 926
- EP-A- 0 195 550
- EP-A- 0 202 780
- EP-A- 0 213 799
- EP-A- 0 227 305
- US-A- 4 043 952

## Description

It is well known to absorb aqueous fluids by means of water absorbent particulate polymeric material. In practice the material is always supplied for this purpose as a substantially dry powder that is sufficiently large as to avoid dusting problems. For instance its particle size is typically in the range 75µm up to 3mm.

The polymer can be semi-synthetic and it can be film forming, e.g., as in US-A- 3,935,099. Alternatively it can be wholly synthetic and non-film forming, as in EP-A- 195550. In particular there is described in that specification a process in which a wet particulate mass which is not crumbly is converted to a crumbly state by mixing into the mass polymer particles that are substantially non-sticky when swollen with water and which are non-film forming and which are based on cross linked polyacrylic acid, optionally blended with acrylamide and other monomers. Although that specification mentioned the use of particles as small as 10µm it recommended values above 50µm so as to avoid dusting problems, i.e., as is conventional.

We have also observed that, at any particular rate of addition, decreasing the particle size below the typical minimum of around 100µm tends to make the crumbly mass less friable. This is probably because the smaller particle size results in a greatly increased number of particles. Although the particles are substantially non-sticky when several of the swollen polymer particles contact one another there can be a tendency for them to aggregate. The use of particles as low as 50µm or less is therefore generally undesirable, but a tendency with the use of larger particles, e.g., 200µm and above, is that their rate of absorption of liquid from the environment can be rather slow and, if such particles aggregate, then the aggregates are rather large and this can be undesirable.

According to the invention, a wet particulate sticky mass is converted to a crumbly or flowable solid by mixing into the mass water absorbent polymer particles that are substantially non-sticky when swollen with water and that are non-film forming and that are non-film forming and in this process the particles have an effective dry size within the mass of at least 90% by weight below 50µm and the particles are mixed into the mass while the particles are in the form either of internally bonded friable aggregates having a dry size of at least 90% by weight above 50µm or in the form of a dispersion in water immiscible liquid of particles having a dry size of at least 90% by weight below 50µm.

Thus in one aspect of the invention the polymer is introduced into the sticky mass in the form of a dispersion in water immiscible liquid of polymer particles having a dry size below 50µm. It might have been thought that the incorporation of the water immiscible liquid would be undesirable but this does not seem to be the case and, instead, the liquid serves as a convenient vehicle for introducing the small particles in such a way as to avoid dusting and clustering of the individual particles within the mass. The particles can be mixed into the mass relatively easily so as to obtain uniform distribution of the particles, and they absorb water from the mass very rapidly.

In the second aspect of the invention the particles are introduced as dry powder having a particle size above 50µm and which consists of internally bonded aggregates of finer particles having a size of below 50µm and often below 30µm. For instance polymer gel fines, e.g., as obtained from the comminution of polymer gel or as fines from a reverse phase bead polymerisation process, can be aggregated by swelling with sufficient water to form a comminutable gel, comminuted to a coarse size and dried (e.g., by a fluidised bed). These internally bonded aggregates appear to behave initially as coarse particles and then to behave as fines.

Any aqueous solution that permits swelling can be used. Water is usually best. An aqueous solution of a small amount of a soluble polymer or other binder could be used. The comminution can be to >90% by weight above 50µm and usually above 100µm, but generally below 1 or 2mm and often below 500µm. Comminution can be by conventional gel comminution methods. Drying can be by conventional techniques followed if necessary by comminution in conventional manner. The resultant aggregates have a size in the range generally of 50 to 500µm. They can very satisfactorily be used in the invention. The fines within each aggregate typically have a size mainly 5 to 30µm and often below 20µm.

By swelling the fines into a comminutable gel, the resultant dried comminuted particles appear to be internally bonded. This is in contrast to the skin bonding effect that is obtained if fines are merely sprayed with water and immediately dried in a fluid bed. Skin bonded aggregates can be used in the invention but internally bonded aggregates give better results. They are novel materials. By this means it is possible to achieve the rapid uptake of water and good friability at low doses that is obtained with the use of fine particles while avoiding the dusting problems and the risk of reduced friability at excess dosages that occurs with fine particles. Particularly good friability can be obtained, without risk of overdosing, using these aggregates. Preferably at least 90% by weight of the aggregates are above 125µm.

The wet particulate sticky mass may be organic, for instance food waste or sewage, but is generally inorganic. It may be, for instance, sand, china clay, crushed mineral, red mud deposits, phosphate slime or coal. The process is of particular value when the particulate sticky mass is environmentally important, e.g., toxic or semi-liquid industrial waste, when it is economically important, e.g., carbon black or metallurgical suspension such as red mud or copper concentrates. The particulate material can be hydrophilic but is preferably hydrophobic.

The invention is of particular value when the sticky mass is a coal fines filter cake, for instance the sticky mass that results from vacuum filtration by a disc, drum or other vacuum filter of a slurry or froth flotation concentrate of coal fines, typically having a particle size below 0.5mm. Often the particle size is mainly in range 50 to 300µm, often at least 80% by weight below 100µm. The ash content of the cake is usually below 30% often below 15%. The cake can be taken direct from the filter or it can be stored for prolonged periods, e.g., as a wet coal fine dump, before treatment in the invention.

The resultant mass is crumbly, as opposed to the sticky and pasty texture before treatment, and can easily be mixed with coal smalls to form a useful fuel, or used in some other way. Whereas 10% coal fines is often the maximum that can be incorporated by traditional techniques, in the invention the amount of coal fines can be increased considerably, e.g., to 20% or more. Typically the crumbly dry coal fines are used as an industrial fuel, e.g., in an electricity generating station. Often they are subjected to various treatments, such as blending, pelleting and/or grinding, before being burnt.

The coal fines filter cake or other wet particulate mass generally has a water content in the range 15 to 50%, often 20 to 40% and usually around 25 to 35%.

It is necessary to ensure uniform mixing of the polymer particles into the sticky mass. The mixing generally comprises some degree of back mixing and, in particular, plug mixing should be avoided since it will result in parts of the sticky mass remaining sticky, due to inadequate contact with polymer particles. The mixing can be achieved by tumbling the mass but preferably it is by means of a rotating mixing blade or other mixer that provides adequate shear. Preferably the mixing is by a Simon or other double scroll mixer or, preferably a plough share mixer, for instance a Lodige or Morton mixer. A plough share mixer has a substantially horizontal cylindrical container provided with a coaxial rotating shaft that carries a plurality of mixing shovels each generally having the shape of a plough share and mounted to rotate close to the wall of the cylinder. The peripheral speed and shape of the shovels causes the product to be whirled from the particulate mass in the lower part of the cylinder into the free mixing zone above the mass, so as to obtain high turbulence and both forward and back mixing.

The polymer must not become sufficiently sticky during the process to cause permanent aggregation of the particles that are being treated. The polymer preferably is wholly insoluble. If, as is preferred, the polymer is a synthetic polymer then the polymerisation conditions and the monomers are preferably such that the content of high molecular weight linear, or soluble, polymer is sufficiently low that during the process the particles do not become sticky.

The polymer may be natural or modified natural polymer such as a starch acrylonitrile graft copolymer or other modified starch, but preferably it is a synthetic polymer. It may be formed from a monomer blend such that the polymer, in linear form, is swellable but insoluble, for instance as a result of including hydrophobic monomer in the monomer blend. Such polymers can, for instance, be made by oil-in-water emulsion polymerisation. For instance they may be made at a pH at which they are relatively non-swellable and insoluble and the pH may then be adjusted, for use, to a value at which the particles are swellable and absorbent and that is the pH of the wet particulate mass.

Generally however the polymer is made from water soluble monomer or monomer blend. Suitable monomers are generally monoethylenically unsaturated monomers but cross linking agent is preferably included in order to convert the resultant polymer to water insoluble but water swellable form. The cross linking agent can be reacted into the polymer after polymerisation but preferably is present during polymerisation. Generally it is a di- or other poly- ethylenically unsaturated monomer such as methylene bis acrylamide or any of the other ethylenically unsaturated cross linking agents that are suitable for cross linking absorbent polymer particles. Instead of or in addition to relying on a covalent cross linking agent of this type, cross linking can also be through pendant groups in known manner. For instance it can be by polyvalent metal ions.

When the polymer particles are of cross linked, water swellable but insoluble, synthetic polymer, it is sometimes possible to achieve adequate results using a non-ionic polymer but best results are obtained more reliably using a cationic or anionic polymer. The polymer is made from the appropriate monomer or monomer blend. The monomers are generally acrylic. Preferably 5 to 100%, often 10 to 100% is ionic.

Suitable anionic monomers are ethylenically unsaturated carboxylic or sulphonic monomers such as (meth) acrylic acid, allyl sulphonate or 2-acrylamido melthyl propane sulphonic acid. Anionic monomers are generally present as a water soluble salt, usually a sodium salt.

Suitable non-ionic monomers are (meth) acrylamide and (meth) acrylicesters.

Suitable cationic monomers are dialkyl amino alkyl (metho) -acrylate or -acrylamide as free base, acid salt or, preferably, quaternary salt and diallyl dimethyl ammonium chloride. Cationic monomers are generally used as a blend with acrylamide. Anionic monomers may be present as homopolymer or as copolymers of anionic monomer with, preferably, acrylamide.

The polymers can be as described in EP-A- 213799, or cationic versions thereof.

In some instances best results are achieved using cationic polymer or blends of cationic polymer with anionic polymer, but it is often preferred to use anionic polymer alone. The preferred anionic polymers are cross linked polymers of 5 to 100 mole % acrylic acid (as free acid or salt) with 0 to 95 mole % acrylamide and optionally 0 to 50 mole % other non-ionic or anionic monomer. The acrylic acid is preferably present wholly or mainly, e.g., at least 70 or 80% by weight, as sodium acrylate. Suitable polymers are copolymers in which the amount of acrylic acid (as free acid or salt) is typically from 20 to 75% by weight, with the balance being acrylamide. It is generally preferred for least 40% by weight of the monomers for the anionic polymer to be sodium acrylate. Typical polymers of this general type are cross linked polymers of 40 to 60% by weight sodium acrylate with 60 to 40% by weight acrylamide when used as dispersions in water immiscible liquid.

Particularly preferred swellable polymers for use in the invention are sodium polyacrylate homopolymers, although up to 20% of the sodium acrylate can be replaced by acrylamide. Also some or all of the sodium acrylate groups can be replaced by acrylic acid or by other water soluble salts, generally alkali metal salts.

The degree of swellability and absorption is controlled, in part, by the extent of cross linking and the amount of cross linking agent is usually below 500ppm, often below 300ppm. It is usually at least 10ppm or 20ppm and preferably at least 50ppm. Best results are often achieved at around 100 or 200ppm. These amounts are the amounts by weight of monomer of methylene bis acrylamide and equivalent amounts of other cross linking agents may be used.

The degree of cross linking, and the polymer type, should be such that the gel capacity of the polymer (grams deionised water absorbed per gram polymer) is at least 25, generally at least 100 and preferably at least 200 typically up to 500 or even 700 or higher.

In some instances it is desirable for the polymer particles to have a surface layer that is less swellable than the inner parts of the particles. The desired reduced swellability of the surface layer is preferably obtained by cross linking the surface layer. This reduces the content of linear polymer at any position where it might cause stickiness and has the advantage of promoting uptake of water and of preventing aggregation of the polymer particles. The desired cross linking can be achieved by methods such as those described in US-A-3,114,651, 3,251,814, 4,043,952, and 4,090,013, JP-A-5842602 and EP-A-227305. Other ways of treating the surface are by applying a coating of a counter ionic polymer (e.g., poly diallyl dimethyl ammonium chloride or other cationic polymer when the swellable polymer is anionic) or by applying sodium aluminate or other aluminate.

The polymer particles may be introduced as individual particles having the size that is required during the mixing step or they may be introduced as aggregates that we assume break down during the mixing step into smaller particles.

When the particles are introduced into the mixing step in the form of a dispersion in water immiscible liquid, preferably at least 90% of the particles are below about 20µm or 30µm, and most preferably below 10µm. Fastest results are generally achieved with at least 90%, preferably 99%, by weight being below 3µm, e.g., in the range 0.03 to 2µm. Often however adequate results are obtained in a cost effective manner, albeit more slowly, if the particle are 90% between 5 and 50µm, e.g., about 5 to 30µm.

Wheras most industrial processes that use dispersions of polymer in water-immiscible liquid require that the amount of polymer should be as high as possible, in the invention we find that best results are achieved when the amount of polymer is relatively low. Thus although the dry weight of polymer can be up to, for instance, 50 or 60% by weight of the dispersion, the dry weight of polymer in the dispersion is preferably below 45% by weight and preferably below 40%. Generally it is at least 15%, preferably at least 20%. Concentrations of 30 to 40% polymer dry weight based on total dispersion are often best when the polymer particles are wet and 20 to 30% when the polymer particles are dry.

The water-immiscible liquid may be any organic liquid in which the polymer particles can be adequately dispersed and that will not interfere with the process and so in practice needs to be substantially water immiscible. It can be, for instance, a vegetable oil but is preferably a hydrocarbon or halogenated hydrocarbon liquid. It may be selected from any of the liquids conventionally used in reverse phase dispersions. For instance it can be kerosene or diesel oil or other mineral oil.

The dispersion can be formed at the point of use, with the polymer particles being dispersed into the water-immiscible liquid and the mixture then being applied substantially immediately to the wet particulate mass. Preferably however the disperson is preformed, in which event it needs to be substantially stable against settlement.

One form of dispersion is a suspension obtained by dispersing preformed dry polymer particles into water-immiscible liquid in the presence of a dispersion stabiliser. The preformed dry polymer particles can be reverse phase microbeads but preferably they are fines separated from polymer gel, e.g., obtained during the comminution of bulk or bead gel or separated from beads obtained by reverse phase polymerisation.

The amount of stabiliser is generally from 1 to 15%, often 3 to 10%, by weight based on the dry weight of polymer. Conventional stabilisers for oil based dispersions may be used, e.g., Bentone clays but preferably the dispersion is stabilised by stirring into it an aqueous emulsion of an oil soluble or oil swellable polymeric thickener, generally a thickener that is insoluble and non-swellable in water. Suitable thickeners are described in EP-A-0161926, for instance in Example 7 and at page 11 line 22 to page 12 line 10.

Instead of using polymer fines, typically having a size of 10 to 30 or 10 to 40µm, the dispersion can be a reverse phase dispersion made by reverse phase polymerisation of aqueous monomer of monomer blend in water-immiscible liquid. See for instance US-A- 4,059,552. The reverse phase polymerisation is preferably conducted as a reverse phase suspension polymerisation. Formation of an initial dispersion of monomer particles can be facilitated by the incorporation of a small amount of water-in-oil emulsifying agent. Often amphipathic stabiliser is included, in known manner, especially when the dispersion is subsequently azeotroped. Depending upon the degree of agitation when forming the initial dispersion of aqueous monomer in the non-aqueous liquid, and depending upon the amount and type of stabiliser and emulsifier, if present, the dry particle size of the final dispersion can be controlled and typically has a maximum size of 1µm or up to 2 or 3µm or 10µm at the most. The product of the reverse phase polymerisation can be described as an emulsion. It may be dried, e.g., by azeotroping to reduce the water content, typically to below 15% by weight of the polymer. The product is then a substantially dry dispersion.

The amount of amphipathic stabiliser (if present) is generally in the range 0.2 or 0.5 to 10%, and generally below 5%, based on the weight of polymer. The amount of water-in-oil emulsifier is preferably from 0.2 to 3%, based on weight of monomer.

In normal processes in which a reverse phase dispersion in oil of water soluble or swellable polymer is mixed into water, it is conventional to conduct the mixing in the presence of an oil-in-water emulsifier so as to promote distribution of the dispersion and the dispersed polymer into the water. For instance, it is common to add the emulsifier to the polymer dispersion before blending with the water. Because of the apparent need to achieve rapid distribution of the polymer throughout the wet particulate mass, we therefore expect it to be necessary to use such an emulsifier. We have surprisingly found, in the invention, that better results are achieved in the absence of this emulsifier than when the conventional addition is made. This suggests, surprisingly, that it is desirable to retard the rate at which the polymer particles are made available to, and can take up water from, the wet particulate mass.

Since one purpose of the polymer particles is to absorb water from the wet particulate mass it would be expected that the particles should be as dry as possible at the start of the process. However we have surprisingly found that improved results are achieved when, at the time of addition to the wet particulate mass, the polymer particles in the dispersion contain a substantial amount of water, usually at least 30% based on the dry weight of polymer. Usually the amount is below 150% and typically is in the range 60 to 120%, preferably 80 to 100%, based on the dry weight of polymer.

Preferred composition comprise 20 to 50% by weight of each of the polymer (dry weight), water-immiscible liquid and water. The amount of each of the polymer and the water immiscible liquid is preferably 25 to 45%, most preferably 30 to 40% by weight. The amount of the water is preferably from 20 to 40%, most preferably 25 to 35%. Particularly preferred compositions comprise 30 to 40% by weight polymer, 30 to 40% by weight water immiscible liquid and 25 to 35% by weight water, with the amount of water generally being less than the weight of polymer.

Compositions containing such amounts of water tend to be unstable if the dry particle size is significantly above 10µm and so the preferred composition that contain water have a particle size lower than this, preferably below 3µm. They can be made by reverse phase polymerisation (usually by reverse phase suspension polymerisation) to form an emulsion of aqueous polymer gel particles dispersed in the water immiscible liquid, and then the emulsion can be used as water without further drying and without the addition of oil-in-water activator. However for some purposes it appears best to dry the emulsion by azeotroping in conventional manner and then to add water back into the dispersion.

It is very surprising that better results can be achieved using wet polymer particles than dry, both because it would be expected that dry particles would be more effective absorbents and because it has occasionally been suggested in the literature that wet particles initiate absorption quicker than dry particles. However the improved results obtainable in the absence of oil-in-water emulsifier indicate that accelerated absorption is not desirable.

When the polymer particles are large, such that the swollen polymer particles have a size greater than the size of most or all of the particles being treated, the swollen polymer particles can subsequently be separated from the dry treated particles. For instance in one process according to the invention at least 50% (dry weight) of the swollen polymer particles have a size greater than the size of at least 95% of the substantially dry treated particles, and these oversize swollen particles are separated from the dry treated particles. Preferably the polymer particles swell to at least twice their dry diameter and substantially all the said swollen polymer particles have a size greater than the size of substantially all the dry treated particles and the polymer particles are separated from the dry treated particles. The separation may be by conventional size classification or weight classification techniques, preferably by seiving using a vibrating seive.

When the particles being treated are coal fines, the resultant friable mass is subsequently used as fuel and as a result of having separated the polymer from the fines the water content of the polymer is not carried in to the fuel and the separated swollen particles can, if desired, be dried (e.g., by heat exchange from the fuel burner) and can be recycled for further use.

The swellable polymer particles may be mixed with the wet particulate mass without any prior addition of any material to the particulate mass. However improved results can be achieved if the particulate mass that is mixed with the swellable polymer particles has previously been treated with a co-ionic dispersing agent, a counter-ionic coagulant, or a co-ionic, counter-ionic or non-ionic flocculant. For instance the mass may be blended with a solution of the dispersing agent, coagulant or flocculant so as to promote liberation of bound water from the cake, before adding the absorbent polymer particles. In some instances it can be desirable to include the dissolved agent with the mass at the time of a filtration stage, e.g., for producing the mass as a wet filter cake. For instance a slurry or froth concentrate of coal fines can be treated by a coagulant or a flocculant or a combination (usually a coagulant followed by a flocculant) prior to filtration to provide the wet filter cake.

Co-ionic dispersing agent is generally a polymer of low molecular weight, usually below 500,000, generally below 200,000 and often below 50,000. For many processes molecular weights of below 10,000, e.g., 2,000 to 5,000, are satisfactory. The dispersing agent is usually anionic. The counter-ionic coagulant generally has a molecular weight of above 50,000, often in the range 100,000 to 1 million, typically about 500,000. However it can have a higher molecular weight. The flocculant can have molecular weight below 1 million but generally it is above. It can be of several million, and can be of typical flocculant molecular weight.

Although these polymeric agents are usually substantially linear and in true solution, it can be particularly advantageous, when the agent is a higher molecular weight agent such as a flocculant, for it to be in the form of very small particles at the time it is mixed with the wet mass, preferably being a slightly cross linked polymer, as described in EP-A- 0202780.

The added agents are usually synthetic polymers formed from water soluble ethylenically unsaturated monomers, and these monomers will be chosen to give the polymer the desired ionic characteristic. Generally the agents are formed wholly from ionic monomers or from blends of ionic monomers with acrylamide or other non-ionic monomers, such as (meth) acrylic esters.

The anionic monomer is preferably acrylic acid but can be any other suitable ethylenically unsaturated monocarboxylic acid or sulphonic acid. It can include or consist of 2-acrylamido-2-methyl propane sulphonic acid. The anionic monomer is generally present as a water soluble salt, generally the sodium salt.

Suitable cationic monomers include diallyl dimethyl ammonium chloride and dialkyl amino alkyl (meth) -acrylates or -acrylamides, generally as acid addition or quaternary ammonium salts. For instance the cationic dispersing agent is preferably a low molecular weight polymer of diallyl dimethyl ammonium chloride or dimethyl amino ethyl (meth) acrylate, or a blend of either of these with acrylamide.

When a dispersant or coagulant or other material is being incorporated before the absorbent polymer, it is generally applied as a solution but can be applied in solid form if its solubility is such as to permit it to dissolve relatively rapidly within the wet filter cake.

It is often preferred that the particle sizes and the amounts of the absorbent polymer and of the filter cake are such that the number ratio of polymer particles:filter cake particles is approximately 1, e.g., from 3:1 to 1:3. For instance this is achieved by adding about 0.2% (dry on dry) of polymer particles having a particle size of about 20 to 30µm to filter cake having a particle size of about 100µm. Larger amounts of these polymer particles are appropriate when the filter cake has a significant electrolyte content.

The amount of polymer that is applied is generally at least 0.005% and is preferably at least 0.05%. It is usually below 5%, preferably below 1% and most preferably is around 0.05 to 0.5%. It is a particular advantage of the invention that, despite the unpleasant character of the wet mass, good results can be obtained with very low amounts of polymer, often below 0.3% or 0.4% and often below 0.15% or 0.2%. These amounts are of dry polymer based on dry particles by weight.

The following are some examples. The coal filter cakes used in these examples have a maximum particles size below 0.5mm and contain generally 20 to 30% water and 10 to 15% ash. In the examples values are named as the "shear dissocciation time" and the "dissociation time".

The "dissociation time" is recorded by putting 600g of the coal filter cake in a Hobart mixer bowl, adding the water absorbent polymer, and stirring at speed 2 until the product became sufficiently friable that aggregates start being thrown out of the bowl. The time take for this stage to be reached is the dissociation time and should be as low as possible.

After stirring for a further 2 minutes at speed 1, the resultant mix is left for 30 minutes in a sealed bag. 100 grams of the mix is put into a cylinder 65mm in diameter and pressed into this cylinder to a disc under a cake-forming pressure of 0.38kg/cm² (5.5psi) to give a cake. The cake is placed on a rectangular plate so that the entire cake is within the profile of the plate, but a substantially semicircular portion is cut away from one side of the plate so that about one third of the cake is unsupported. A solid plate is lowered at 12mm/sec on to the top of the cake by a piston and is pressed down on to it with a pressure of 5psi (0.35kg/cm²). The time is measured between the plate touching the top of the cake and the cake shattering over the cut away part of the test plate. This is the shear dissociation time (SDT 5). If the cake shatters immediately upon contact with the lowering plate, the shear dissociation time is recorded as zero. Again, low values are preferred. The test can be repeated at higher cake-forming pressures of 20 and 50 psi to give SDT 20 and SDT 50 values.

SDT 5 needs to be below 30 seconds for generally satisfactory results and, in particular, if SDT 5 is below about 20 seconds, preferably below about 10 seconds and most preferably below about 7 seconds (especially substantially zero) and if the dissociation time is satisfactory, then the polymer cake combination is such that, with appropriate mixing, homogeneous blendability with coal smells can be expected. For instance Examples 1 and 2 below show that good results are obtained when SDT 5 is not above 7 and dissociation is not above 18.

For the friable cake to resist caking or clogging during transport, a more friable texture is needed. For this, the SDT test is repeated under a cake-forming pressure of about 20 psi (1.4kg/cm²), to determine SDT 20, or even at about 50psi (3.5kg/cm²) to determine SDT 50. These values also should be below about 20, preferably below about 10, most preferably below about 7 seconds, especially substantially zero.

### Example 1

Sodium polyacrylate cross linked with 0.025% methylene bis acrylamide is formed by conventional bulk gel polymerisation and is dried and comminuted in conventional manner. The resultant particles are classsified according to size and the fines are retained for use in the invention. They have a dry particle size below 50µm, mainly in the range 10 to 30µm.

The fines are dispersed into an equal weight of a hydrocarbon oil that is thickened with a dispersion stabiliser as described at page 18 lines 25 to 35 of EP-A-0161926. 1% oil-in-water emulsifier is included.

The dispersion is sprayed on to a wet filter cake of coal fines, this filter cake having been taken from a vacuum filter following froth flotation. The amount of dispersion is 0.1% dry polymer on dry particulate mass. The product is mixed thoroughly and rapidly became a friable, crumbly solid. This can easily be blended with coal smalls to form a fuel. Without the addition of the dispersion, the filter cake is a wet sticky mass that could not easily be used.

In a comparison, when a similar amount of dry polymer particles of the same polymer but having a size of around 100µm, and that are not dispersed in oil, was added to the cake, the cake does not become so crumbly so quickly. With prolonged mixing and larger amounts of polymer (.e.g, 0.2% or even 0.5%) the product is adequately crumbly but swollen polymer particles and aggregates are apparent.

### Example 2

Three types of dispersion, each containing equal amounts of polymer and hydrocarbon oil (kerosene or diesel), and oil-in-water emulsifier, are made as follows.

Suspensions - the general technique of Example 1 using particles of the size shown, with >90% by weight <50µm when the suspension is shown as <65µm

RP Emulsions - by the reverse phase polymerisation to give a product of about 35% oil, 35% polymer, 30% water

RP Dispersions - by azeotroping RP Emulsions to about 50% polymer 50% oil

The compositions are tested at 0.5% product on wet coal filter cake as above. The monomers used and the results are in the following table, where NaAc = % sodium acrylate, ACM = % acrylamide and MBA = methylene bis acrylamide (ppm).

It is apparent from this that the overall trend is that better results are obtained when the size is below 50µm. The disadvantage of too little cross-linking agent, for the particular mass, is apparent. This is probably due to the polymer containing too much soluble polymer.

### Example 3

Tests similar to Example 2 are conducted on RP dispersions of 50% oil and 50% of a copolymer of 50% NaAc 50% ACM 200 ppm MBA with or without added oil-in-water emulsifier, at different amounts of polymer.

The disadvantage of incorporating emulsifier is apparent.

### Example 4

Tests similar to Example 2 are conducted on a 50% RP dispersion of a copolymer of 50% NaAc 50% ACM 200 ppm MBA (product A) and the same product after dilution to 25% polymer by red diesel oil (B).

The benefit of reducing the polymer concentration is apparent.

### Example 5

A RP dispersion is formed of 50% oil 50% copolymer of 50% NaAc 50% ACM 200 ppm MBA. This is diluted with various amounts of water and the products are tested on wet coal filter cake as in Example 2 at different dosages of product.

This clearly shows that the addition of a controlled amount of water gives improved results at low dosages and thus provides a particulary cost effective system.

### Example 6

Example 2 is repeated using similar amounts of three different polymer suspensions. ACN is acrylonitrile.

Tests 5, 6 and 7 were conducted with different starch acrylonitrile copolymers dispersions. Tests 8-10 are with 60% dispersions in oil and tests 11 to 13 are with 50% dispersions in oil. Tests 14 is with 1% of a 25% emulsion of aqueous polymer particles in oil and test 15 with a 50% dry dispersion of similar, but dry, polymer particles.

### Example 8

The process of example 2 is repeated but using a 35% by weight RP emulsion in oil of cationic swellable polymer formed from 60% ACM 40% dimethylaminoethyl acrylate (MeCl quaternary salt). At 1% dosage, Dissociation is 11.7 seconds and SDT 5 is 0.9. When using a 1% polymer dosage of a 50% RP dispersion of a swellable polymer of 50% ACM 50% NaAc (instead of the cationic polymer). Dissociation is 11 and SDT 5 is 1.2.

### Example 9

An aqueous solution of cationic soluble polymer A. B or C is stirred into a wet filter cake of coal fines. After stirring for one minute, a 50% dispersion in oil of cross linked gel polymer particles of acrylamide and sodium acrylate polymer is blended into the filter cake. The results are as follows, in which polymer A is a low molecular weight diallyl dimethyl ammonium chloride coagulant, polymer B is a high molecular weight, slightly cross linked, copolymer of 59 mole percent acrylamide and 42 mole percent cationic dialkylaminoalkyl acrylate quaternary monomer, and polymer C is a homopolymer of a cationic dialkylaminoalkyl methacrylate quaternary monomer. In addition to the results shown in the table below, the product was assessed visually and it was significant that increasing amounts of product B, and especially the tests with product C, gave the best visual appearance.

### Example 10

Fines having a size mainly 10-30µm are separated from comminuted cross linked polyacrylic acid (75% as sodium salt) gel having a gel capacity well in excess of 25g/g. They are labelled A. Part of them are mixed with sufficient water to make a comminutable gel which is then comminuted and dried on a fluid bed drier, in conventional manner, to a particle size >125µm but below 500µm. This is labelled B. Each product is mixed with coal filter cake as in Example 1 at various doses.

This demonstrates that the agglomerates give improved results at higher dosages but give similar results at lower dosages.

As a comparison products A, B and C are formed from 50% ACM 50% NaAc cross linked swellable polymer having gel capacity above 25g/g. A is a dispersion in oil of particles <40µm. B is powder <63µm and C >125µm. Different amounts are blended as in Example 1. The results are as follows.

### Example 11

Polyacrylic acid (about 75% in sodium form) gel cross linked with about 200ppm MBA is formed, comminuted and dried in conventional manner. Fines having a size mainly in the range 10 to 40µm are separated and dispersed at 50% solids in kerosene or diesel using an emulsion of stabilising polymer (as in EP-A-0161926, Example 7) as stabiliser.

The resultant dispersion is diluted to about 25% solids with further kerosene or diesel and sprayed at about 0.2% polymer on to coal filter cake having a coal size mainly 50 to 150µm and a moisture content around 30% and an ash content of around 10% as the cake is fed into a continuously moving Lodige Plough Share mixer.

The mix passes through the mixer in not more than about 2 minutes and emerges as a friable product that can easily be crumbled between the fingers (the SDT 5 for the wet filter cake-polymer combination is below 10).

The friable product is blended with about 5 times its own weight of coal smalls having a size of 1 to 10mm and the mix is pulverised and carried, entrained in air from the pulverisers, as a fuel into the combustion chamber of a power station boiler. There is no evidence of clogging of the pulverisers or other parts of the apparatus through which the product travels from the mixer to the boiler.

The blend, before pulverisation, may flow evenly out of a Durham Cone at that is uniform and is about 1.4kg/sec, whereas the untreated cake clogs or flows unevenly at about half that rate.

### Example 12

A wet cake of particulate magnetite having 14.6% moisture content is blended with a dispersion in oil of swellable, cross-linked polymer fines having a particle size below 40µm. The amount of dispersion is 0.25% by weight polymer based on wet magnetite. When the polymer is formed from 50% ACM 50% NaAc, dissociation time = 7 seconds, SDT 5 = 0 and SDT 20 > 30. When the polymer is formed of neutralised polyacrylic acid, dissociation time = 8.2 seconds, SDT 5 = 5.7 and SDT 20 > 30.

## Claims

1. A process in which a wet particulate sticky mass is converted to a crumbly or flowable solid by mixing into the mass water absorbent polymer particles that are substantially non-sticky when swollen with water and that are non-film forming, characterised in that the particles have an effective dry size within the mixture of at least 90% below 50µm and are mixed into the mass while the particles are in the form either of internally bonded friable aggregates of above 50µm in size formed of particles below 50µm in size, or of a dispersion in water immiscible liquid of particles below 50µm in size.

2. A process according to claim 1 in which the polymer is a cross linked polymer formed from anionic or cationic ethylenically unsaturated monomer optionally mixed with non-ionic monomer, and has gel capacity of at least 25g/g.

3. A process according to claim 2 in which the polymer is a cross linked polymer of 80 to 100% acrylic acid sodium salt and 0 to 20% acrylamide.

4. A process according to any preceding claim in which the surface of the polymer particles is preferentially cross linked.

5. A process according to any preceding claim in which the particles have at least 90% by weight below 50µm and are added to the mass while present as a dispersion in water immiscible liquid of particles below 50µm in size.

6. A process according to claim 5 in which the dispersion is a dispersion of fines obtained from polymer gel.

7. A process according to claim 6 in which the dispersion is stabilised against settlement as a result of the incorporation into the dispersion of an oil swellable or oil soluble polymeric thickener.

8. A process according to claim 5 in which at least 90% by weight of the polymer particles have a dry size below 10µm and the dispersion has been obtained by reverse phase polymerisation.

9. A process according to any of claims 5 to 8 in which at least 90% by weight of the particles have a dry size below 10µm and a dispersion contains at least 30% by weight water.

10. A process according to claim 9 in which the dispersion is made by reverse phase polymerisation and comprises 25 to 45% by weight of the polymer particles, 20 to 40% by weight water and 25 to 45% by weight water immiscible liquid.

11. A process according to any of claims 5 to 10 in which the dispersion is substantially free of oil-in-water emulsifier.

12. A process according to any of claims 1 to 4 in which the particles are introduced as internally bonded aggregates having 90% by weight above 125µm of particles below 40µm in size.

13. A process according to claim 12 in which SDT 20, the shear dissociation time at 20 psi (1.4 kg/cm²), is below 10.

14. A process according to any preceding claim in which the mixing provides both forward and back mixing.

15. A process according to any preceding claim in which the mixing is conducted by a double scroll or plough share mixer.

16. A process according to any preceding claim in which the particulate polymeric material, its amount and the particulate mass are such that SDT 5, the shear dissociation time at 5 psi (0.35 kg/cm²) is below 20 and dissociation time is below 50.

## Patentansprüche

1. Verfahren, bei welchen eine nasse, feinteilige, klebrige Masse in einen krümeligen oder fließfähigen Feststoff umgewandelt wird, indem man in die Masse wasserabsorbierende Polymerteilchen einmischt, die nach dem Quellen mit Wasser praktisch nicht klebrig und nicht filmbildend sind, dadurch gekennzeichnet, daß mindestens 90 % der Teilchen innerhalb der Mischung eine effektive Trockengröße von weniger als 50 µm haben und die Teilchen, während sie in die Masse eingemischt werden, entweder in Form innerlich gebundener, bröckeliger Aggregate einer Größe über 50 µm, gebildet aus Teilchen einer Größe unter 50 µm, oder in Form einer Dispersion von Teilchen einer Größe unter 50 µm in einer mit Wasser nicht mischbaren Flüssigkeit vorliegen.

2. Verfahren gemäß Anspruch 1, bei welchem das Polymer ein vernetztes Polymer ist, das aus einem anionischen oder kationischen, ethylenisch ungesättigten Monomer, gegebenenfalls mit einem nicht ionischen Monomer gemischt, gebildet ist und eine Gelkapazität von mindestens 25 g/g hat.

3. Verfahren gemäß Anspruch 2, bei dem das Polymer ein vernetztes Polymer aus 80 bis 100 % Acrylsäure-Natriumsalz und 0 bis 20 % Acrylamid ist.

4. Verfahren gemäß irgendeinem vorhergehenden Anspruch, bei dem die Oberfläche der Polymerteilchen vorzugsweise vernetzt ist.

5. Verfahren gemäß irgendeinem vorhergehenden Anspruch, bei dem mindestens 90 Gew.-% der Teilchen eine Größe unter 50 µm haben und der Masse zugefügt werden, während sie als Dispersion aus Teilchen einer Größe unter 50 µm in einer mit Wasser nicht mischbaren Flüssigkeit vorliegen.

6. Verfahren gemäß Anspruch 5, bei dem die Dispersion eine Dispersion aus Feinstoffen ist, die aus Polymergel erhalten wurden.

7. Verfahren gemäß Anspruch 6, bei dem die Dispersion gegen ein Absetzen aufgrund der Einverleibung eines mit Öl quellfähigen oder öllöslichen polymeren Verdickungsmittels in die Dispersion stabilisiert ist.

8. Verfahren gemäß Anspruch 5, bei dem mindestens 90 Gew.-% der Polymerteilchen eine Trockengröße unter 10 µm haben und die Dispersion durch Umkehrphasen-Polymerisation erhalten worden ist.

9. Verfahren gemäß irgendeinem der Ansprüche 5 bis 8, bei dem mindestens 90 Gew.-% der Teilchen eine Trockengröße unterhalb 10 µm haben und die Dispersion mindestens 30 Gew.-% Wasser enthält.

10. Verfahren gemäß Anspruch 9, bei dem die Dispersion durch Umkehrphasen-Polymerisation hergestellt ist und 25 bis 45 Gew.-% Polymerteilchen, 20 bis 40 Gew.-% Wasser und 25 bis 45 Gew.-% mit Wasser nicht mischbare Flüssigkeit umfaßt.

11. Verfahren gemäß irgendeinem der Ansprüche 5 bis 10, bei dem die Dispersion von einem Öl-in-Wasser-Emulgator im wesentlichen frei ist.

12. Verfahren gemäß irgendeinem der Ansprüche 1 bis 4, bei dem die Teilchen als innerlich gebundene Aggregate mit einer Größe von zu 90 Gew.-% über 125 µm eingeführt werden, wobei die einzelnen Teilchen eine Größe unter 40 µm besitzen.

13. Verfahren gemäß Anspruch 12, bei dem SDT 20, d.h. die Scherdissoziationszeit bei 20 psi (1,4 kg/cm²), unter 10 liegt.

14. Verfahren gemäß irgendeinem vorhergehenden Anspruch, bei dem das Mischen sowohl ein Vorwärts- als auch Rückwärtsmischen vorsieht.

15. Verfahren gemäß irgendeinem vorhergehenden Anspruch, bei dem das Mischen durch einen Mischer mit doppeltem Kronenrad oder einen Pflugscharmischer erfolgt.

16. Verfahren gemäß irgendeinem vorhergehenden Anspruch, bei dem das feinteilige polymere Material, seine Menge und die feinteilige Masse so bemessen sind, daß SDT 5, die Scherdissoziationszeit bei 5 psi (0,35 kg/cm²), unter 20 und die Dissoziationszeit unter 50 ist.

## Revendications

1. Un procédé dans lequel une masse collante particulaire humide est transformée en un solide friable ou fluide en mélangeant dans la masse des particules de polymère absorbant l'eau qui sont pratiquement non collantes lorsqu'elles sont gonflées par l'eau et qui sont non filmogènes, caractérisé en ce que les particules ont une dimension efficace à sec dans le mélange d'au moins 90 % de moins de 50 µm et sont mélangées dans la masse tandis que les particules sont sous la forme soit d'aggrégats friables d'une dimension de plus de 50 µm à liaisons internes formés de particules d'une dimension de moins de 50 µm, soit d'une dispersion dans un liquide non miscible avec l'eau de particules d'une dimension de moins de 50 µm.

2. Un procédé selon la revendication 1, dans lequel le polymère est un polymère réticulé formé d'un monomère éthylénique anionique ou cationique facultativement mélangé avec un monomère non ionique et il a une capacité de gel d'au moins 25 g/g.

3. Un procédé selon la revendication 2, dans lequel le polymère est un polymère réticulé de 80 à 100 % d'acrylate de sodium et 0 à 20 % d'acrylamide.

4. Un procédé selon l'une quelconque des revendications précédentes, dans lequel la surface des particules de polymère est réticulée préférentiellement.

5. Un procédé selon l'une quelconque des revendications précédentes, dans lequel les particules ont au moins 90 % en poids de moins de 50 µm et sont ajoutées à la masse tandis qu'elles sont sous forme d'une dispersion dans un liquide non miscible avec l'eau de particules d'une dimension de moins de 50 µm.

6. Un procédé selon la revendication 5, dans lequel la dispersion est une dispersion de fines obtenues à partir d'un gel de polymère.

7. Un procédé selon la revendication 6, dans lequel la dispersion est stabilisée contre la sédimentation par l'introduction dans la dispersion d'un épaississant polymère gonflable à l'huile ou soluble dans l'huile.

8. Un procédé selon la revendication 5, dans lequel au moins 90 % en poids des particules de polymère ont une dimension à sec de moins de 10 µm et la dispersion a été obtenue par polymérisation à inversion de phase.

9. Un procédé selon l'une quelconque des revendications 5 à 8, dans lequel au moins 90 % en poids des particules ont une dimension à sec de moins de 10 µm et la dispersion contient au moins 30 % en poids d'eau.

10. Un procédé selon la revendication 9, dans lequel la dispersion est faite par polymérisation à inversion de phase et comprend 25 à 45 % en poids des particules de polymère, 20 à 40 % en poids d'eau et 25 à 45 % en poids de liquide non miscible avec l'eau.

11. Un procédé selon l'une quelconque des revendications 5 à 10, dans lequel la dispersion est pratiquement exempte d'émulsifiant huile-dans-l'eau.

12. Un procédé selon l'une quelconque des revendications 1 à 4, dans lequel les particules sont introduites sous forme d'aggrégats à liaisons internes, ayant 90 % en poids de plus de 125 µm, de particules d'une dimension de moins de 40 µm.

13. Un procédé selon la revendication 12, dans lequel le temps de dissociation par cisaillement à 1,4 bar (20 psi), ou SDT 20, est de moins de 10.

14. Un procédé selon l'une quelconque des revendications précédentes, dans lequel le mélange donne à la fois un mélange en avant et à contre-courant.

15. Un procédé selon l'une quelconque des revendications précédentes, dans lequel le mélange est effectué par un mélangeur à double hélices ou à soc.

16. Un procédé selon l'une quelconque des revendications précédentes, dans'lequel la matière polymère particulaire, sa quantité et la masse particulaire sont telles que le temps de dissociation par cisaillement à 0,35 bar (5 psi), ou SDT 5, est de moins de 20 et le temps de dissociation est de moins de 50.
